

April 25, 1939.

C. Q. PAYNE

2,156,125

METHOD OF WET MAGNETIC SEPARATION

Filed March 30, 1937

2 Sheets-Sheet 1



INVENTOR  
CLARENCE Q. PAYNE  
BY  
ATTORNEYS

April 25, 1939.

C. Q. PAYNE

2,156,125

METHOD OF WET MAGNETIC SEPARATION

Filed March 30, 1937

2 Sheets-Sheet 2



## UNITED STATES PATENT OFFICE

2,156,125

## METHOD OF WET MAGNETIC SEPARATION

Clarence Q. Payne, Stamford, Conn.

Application March 30, 1937, Serial No. 133,777

1 Claim. (Cl. 209—214)

This invention relates to a method of wet magnetic separation of ores and minerals, especially those which are finely divided, and is applicable to the separation both of strongly and also of 5 feebly magnetic minerals.

An important object of the invention is to control the gravitational and electrostatic forces which tend to interfere with magnetic attraction exerted on the particles while they are undergoing separation. This is accomplished by feeding the mixed particles in the form of a water diluted feed-stream into a water filled tank, then thickening the feed-stream as it descends to a submerged magnetic field in the tank by removing 10 a practically clear-water over-flow from the top of the tank and at the same time regulating the descent of the thickened pulp by controlling the areas of the discharge outlets for the separated products at the bottom of the tank so that the 15 velocity of descent through the magnetic field will be sufficiently reduced for the deflection of feebly magnetic particles while passing therethrough.

Other objects and advantages of the invention 20 will appear as the description proceeds.

The accompanying drawings show two forms of magnetic separators for carrying out my improved method.

Fig. 1 is a vertical section of a separator which 25 uses a single magnetic field on two flux circuits.

Fig. 2 is a vertical section on the line II—II of Fig. 1.

Fig. 3 is a horizontal section with parts broken away on the line III—III of Fig. 1.

Fig. 4 is an enlarged perspective view of portions of interleaved magnetic and nonmagnetic rotor disks, having open longitudinal grooves along their circumferences.

Fig. 5 is a perspective view of a modified form 35 of magnetic and nonmagnetic disks with longitudinal grooves filled with nonmagnetic material.

Fig. 6 is a vertical section through a modified form of a double-pass separator along the line VI—VI of Fig. 8 having superposed electromagnets, each having two magnetic fields on a single 40 flux circuit.

Fig. 7 is a horizontal section along the line VII—VIII of Fig. 6.

Fig. 8 is a longitudinal sectional elevation on the line VIII—VIII of Fig. 6.

Ores and minerals, especially when finely divided as in the case of clays, slimes, or those crushed to pass about one hundred mesh screen or finer, present serious difficulties to their magnetic separation when they are in the dry state. 55

This may be briefly explained as due to enmeshment or clotting. It may be caused either by absorption of moisture from the atmosphere, or by impressed forces such as an electrostatic charge between minerals of different composition 5 when they are moved upon each other. In either case the effect is to cause adhesion or clotting of the fine particles which prevents their free movement. This causes an inefficient separation of fine magnetic from nonmagnetic particles 10 when they are brought within a magnetic field. Heretofore, wet magnetic separation has been chiefly limited to strongly magnetic iron ores like magnetite. For the most part these have been treated in a coarsely crushed condition, namely, 15 4-8 mesh screen size, or larger. The log-washer type of separator has also been employed in the direct magnetization of finely crushed magnetite ores. In all cases however, free use is made of feed and wash-water to hasten the passage of 20 the ore through the magnetic field.

The purpose of the method of wet separation herein set forth is to greatly enlarge the scope and value of inductive magnetic separation by permitting ores to be treated which have not 25 heretofore been amenable to concentration owing to their extremely fine mineralization. Since water has usually sufficient dissolved salts to make it a good conductor of electricity all clotting of the fine particles from electrostatic charges is 30 overcome when they are submerged in water. This method while capable of exerting the utmost attracting force upon the feed-stream as it passes through the submerged magnetic field-gap is also able to control the velocity of descent of the latter 35 and therefore also the separating force, by eliminating the feed water by overflowing it as it enters the tank in which the separation takes places. Dealing in this way with the regulated speed of subsidence of fine particles in water, it 40 is possible to attract and separate, more easily, those feebly magnetic minerals such as iron silicates, hornblende, biotite, garnet, etc. which can only be acted on when fine, by careful adjustment between the attracting and separating 45 forces. Freedom of motion of the particles among themselves is thus assured, and their effective weight is reduced by the amount of water which they displace. In effect their resistance to separation is thus reduced when submerged. It also 50 permits those tiny occluded and middling particles to be deflected and separated to a much greater degree than has heretofore been possible by means of dry separation.

In the form of magnetic separator illustrated 55

in Figs. 1, 2 and 3, two electromagnets 10 having cores, with like poles, connected by yokes 11 are shown. To these yokes 11, at their central portions, pole pieces 12 are bolted, which carry the 5 magnetic field below the yokes so that a laminated rotor 13 of alternating magnetic and non-magnetic disks may be revolved by means of its shaft 17 below the electromagnets. The shaft 17 is driven from a pulley 18. The laminated disk-rotor 13 forms the armature of the electromagnets and serves also as a separating drum on which the material to be separated is fed from a water filled hopper 19 placed above it. The rotor 13 revolves between concentric faces of 10 the pole pieces 12 with substantially equal gap on each side in order to balance the magnetic attraction of the pole pieces. The width of the field-gap between the pole pieces 12 and rotor 13, in which the separation takes place, is regulated to suit the size of the particles to be separated and is as narrow as practicable to reduce the reluctance of the magnetic circuit. The electromagnets 10 are connected to the current supply so that one yoke will convey only north 15 magnetism to one pole piece, while the other yoke conveys only south magnetism to the other pole piece. In this way a single magnetic field is formed upon two flux circuits as shown by the broken lines and arrows in Fig. 3. The thickness 20 of the magnetic disks 40 and nonmagnetic disks 41 forming the rotor 13 will depend upon the size of the ore particles to be separated. They are provided with horizontal grooves 42 along their circumference in order to increase their 25 holding power by means of the highly convergent magnetized points at the groove intersections as well as at the groove and disk edges themselves, as shown in Fig. 4. These horizontal grooves may be closed by means of nonmagnetic strips 43, as shown in Fig. 5, where it is important to give the rotor a smooth outer surface. The horizontal grooves may also be left open as shown in Fig. 4 where it is desirable to afford some support for the particles undergoing separation as 30 they are carried through the field-gap. The rotor shaft 17 is supported in stuffing-box bearings 20, which are attached to nonmagnetic cheek-plates 21 at each end of the rotor. These fit water tight to the ends of the pole pieces 12 and with the pole pieces form the central portion 35 of the tank in which the separation takes place. It is desirable to protect the surface of the rotor and the faces of the pole pieces with chromium or cadmium plating to prevent rusting. The hopper 19 forming the upper part of the water tank is detachable and has its upper edge surrounded by a continuous trough 22. This enables the overflow from the dilute feed pulp to be collected and discharged to one side. Above the 40 main hopper is a smaller partly submerged V-hopper 23 which is supported upon the upper edge of the main hopper. This smaller feed hopper 23 is of about the same length as that of the rotor, and a plate 24 underlies its discharge opening. The plate 24 deflects the feed-stream of materials to be separated which is discharged in thin sheets 24a towards both sides of the main hopper and enables the feed-water which is introduced with the ore stream, to rise and overflow 45 the top of the main hopper as practically clear water while the thickened pulp descends in a disseminated cloud through the upper part of the tank. It then falls on the inclined guide plates 25 and 26 and is fed to the charged rotor 50

13 which revolves in the direction shown by the arrow in Fig. 1.

The nonmagnetic particles descend along the stationary side of the field gap and fall vertically into a receiving hopper 27. The magnetic particles are attracted and held to the magnetized edges and points of the rotor disks 40 until they are carried over the edge of the division plate 28 when they are released and discharged as they approach the neutral plane of the rotor where all attractive force of the rotor ceases, owing to reversal of polarity. They are then deflected at a divergent angle from the non-magnetic particles and fall vertically on the other side of the division plate into a separate hopper 29 thus effecting their separation from the latter. A brush or scraper 30 serves to dislodge fine steel particles sometimes present in the ore and carried past the neutral line. The receiving hoppers 27 and 29 are bolted water tight to the bottom 20 of the tank which contains the disk rotor. At the discharge ends of these hoppers plug-cocks 31 and 32 are located whose openings can be closely regulated. By varying the openings of these valves 31 and 32 the separated products 25 obtained from the thickened feed-pulp can be discharged either slowly or else rapidly from the separator as the necessity of the material undergoing separation may require. As a further means of regulating and equalizing the velocity 30 of the downward water current through the field-gap it is advisable to provide baffles 33, 34 in the upper part of each of these hoppers.

When the field coils of the electromagnets have been energized to secure the required magnetic flux across the field gap, the rotor is caused to revolve in the direction shown by the arrow. The material to be separated is then fed below the water level of the main hopper tank by means of the small distributing V-hopper 23. The material is thus enabled to free itself more readily from the feed-water which accompanies it and the greater part of the feed water discharges over the top edge of the main tank into the trough 22 as practically clear water. In some cases where 45 the finely ground material is very much diluted, it may be advisable to employ an intermediate settling tank in order to thicken the pulp before feeding it to the separator. In certain cases as in treating clays, it may also be advisable to add 50 an electrolyte to the separator feed tank, such as sodium chloride or caustic starch, in order to remove cloudy suspensions and to hasten the settling of the fine particles. As they descend, the particles are collected by the guide plates 25 and 26 and are fed upon the rotor 13. The magnetic particles are attracted and held to the charged edges and points of the rotor until they are carried over the edge of the division plate 28. The nonmagnetic particles on the other hand 55 pass through the field-gap without being deflected, and are collected in a separate hopper whose discharge rate is controlled by means of the plug-cock 32. In this way and by varying the rate 60 of feed, the speed of the rotor and strength of 65 the field, both the attracting and the separating forces can be brought under closer control than has heretofore been possible, especially in the case of finely divided ores and minerals.

A modification of the design of separator described above and its application to the separation of finely divided materials into three products by means of two superposed electromagnets is illustrated in Figs. 6, 7 and 8. In this form of embodiment of my invention, bipolar electromag- 70 75

nets 50 and 52 are shown in Fig. 6 in their superposed position, each of which has two rotors 51, 51a, 53 and 53a mounted on shafts 56 and 57. These are so assembled with single yokes 54 and 55 that with the aid of keepers 83 and 84 they secure two magnetic fields upon the same flux circuit generated by the electromagnets as shown in Fig. 7. In this design the iron path of the flux circuit can be made somewhat shorter in relation 10 to the length of field-gap available for separation, than in the design shown in Figs. 1, 2 and 3. The two electromagnets 50 and 52 may be energized to produce a clean magnetic concentrate 58 from the top electromagnet 50 and a clean tailings 59 15 and middlings product 60 from the bottom electromagnet 52. The two successive magnetic products may also be combined where they are to be discarded, and where the main object is to secure a clean nonmagnetic product from the 20 crude material by means of a double pass as illustrated in Fig. 6.

The mechanical features in the form of separator illustrated in Figs. 6, 7 and 8 may differ from that illustrated in Figs. 1, 2 and 3 in that 25 the partly submerged V-hopper 61 here has a feed roller 62 underlying its discharge opening in place of plate 24 illustrated in Fig. 1. The feed rollers 62 and 62a revolve with the shaft 63 and deflect the feed-stream of the materials to be 30 separated in such manner that it is discharged in a thin sheet 64 toward the inclined portion 65 of the main hopper. It then falls to the inclined guide plate 66 from which it is fed to the upper charged rotor 51 or 51a which revolves in 35 the direction shown by the arrow in Fig. 6.

The particles which are not attracted by the magnetized edges and points of disks 40 of rotors 51 and 51a fall vertically into the hoppered opening formed by the inclined plates 67 and 68. 40 These are supported above rotors 53 and 53a and guide the particles upon the lower charged rotors 53 and 53a which separate the remaining magnetic particles from the material which has been fed to them. The nonmagnetic portion 45 descends into hopper 69, while the magnetic portion of the material is discharged over the division plate 70 as the rotor 53 or 53a loses its power of attraction at the neutral line due to reversal of polarity.

The particles 58 which have been attracted and deflected by the energized rotors 51 or 51a and carried over division plate 72 may also be 50 collected in hopper 75 along with magnetically attracted particles 68 which have been separated 55 from the nonmagnetic particles 59 by the lower set of rotors 53 or 53a where only two separated products are desired.

The separating rotors in the form illustrated in Figs. 6, 7 and 8 may be revolved by a chain drive connecting the sprocket wheels affixed to the rotor shafts and the counter-shaft 76 which in turn is driven by the pulley 82. Feed-roller shaft 63 is drivably connected to counter-shaft 76 by means of sprocket wheel 77, an endless chain 78 and a sprocket wheel mounted on feed-roller shaft 63. Sprocket wheel 78 which is mounted on counter-shaft 76 is drivably connected with 10 rotor shaft 56 by means of a drive chain 79 and a sprocket wheel mounted on said rotor shaft. Another sprocket wheel mounted on shaft 56 serves to drive rotor shaft 57 with the aid of an 15 endless chain 80 and sprocket wheel 81 mounted on shaft 57. By varying the relative size of these sprocket wheels, the speeds of the various rotors may be varied to suit the nature of the material to be separated.

The principle involved in both the above described designs is, however, the same. The dilute feed-stream is fed into the top of a water filled tank and is thickened as it descends to the submerged magnetic fields by removing a practically clear-water overflow from the top of the 20 tank. The actual separation of the nonmagnetic from the magnetic particles is accomplished by one or more energized rotors, in the tank, while the speed of descent of the thickened feed-stream is controlled by varying the areas of the 25 discharge outlets for the separated products at the bottom of the tank.

I wish it to be understood that my invention is not limited to a combination of the specific elements or to the specific structures illustrated 30 in the drawings, but that it includes all such variations as come within the spirit and scope of the disclosure herein and the claim appended hereinafter.

I claim:

The method of wet magnetic separation of ores and minerals containing feebly magnetic and nonmagnetic particles which consists in submerging them in a tank of water thereby reducing their effective weight, causing the particles of 40 ore to fall through the water and along guide plates into a submerged arcuate magnetic field gap formed between an arcuate faced pole piece and a horizontal magnetic rotor submerged in said tank and attracting the magnetic away from the nonmagnetic particles within said gap by feeding them along the arc of said horizontal rotor in direct contact therewith in said magnetic field, substantially as and for the purpose 45 described.

CLARENCE Q. PAYNE.